

Oct. 26, 1954

P. AUBERT ET AL  
PHOTOGRAPHIC EMULSIONS SENSITIZED WITH MEROCYANINE  
DYES CONTAINING A 5(4)-THIAZOLONE NUCLEUS

2,692,829

Filed Feb. 17, 1951

FIG. 1.



[2-(3-METHYLTHIAZOLINE)][4-(2-ETHYLTHIO-5(4)-THIAZOLONE)] DIMETHINEMEROCYANINE

FIG. 2.



[2-(3-ETHYLBENZOTHIAZOLE)][4-(2-ETHYLTHIO-5(4)-THIAZOLONE)] DIMETHINEMEROCYANINE

FIG. 3.



[2-(3-ETHYLBENZOXAZOLE)][4-(2-ETHYLTHIO-5(4)-THIAZOLONE)] DIMETHINEMEROCYANINE

PER AUBERT  
EDWARD B. KNOTT

INVENTORS

Daniel J. Mayne  
BY Lawrence N. Willis  
ATTORNEY & AGENT

UNITED STATES PATENT OFFICE

2,692,829

# PHOTOGRAPHIC EMULSIONS SENSITIZED WITH MEROCYANINE DYES CONTAINING A 5(4)-THIAZOLONE NUCLEUS

Per Aubert, Oslo, Norway, and Edward B. Knott,  
Harrow, England, assignors to Eastman Kodak  
Company, Rochester, N. Y., a corporation of  
New Jersey

Application February 17, 1951, Serial No. 211,566

18 Claims. (Cl. 95—7)

1

This invention relates to photographic emulsions, methods for making them, and to new non-migratory dyes.

Photographic emulsions containing non-diffusing dyes have been previously described in Brooker U. S. Patent 2,282,116, dated May 5, 1942. The disadvantages attending the use of such dyes resides primarily in their staining properties when the latent image is developed.

We have now found that the prior art deficiencies can be overcome by incorporating in the unexposed photographic silver halide emulsion certain merocyanine dyes.

It is, therefore, an object of our invention to provide new photographic silver halide emulsions. Another object is to provide methods for obtaining these new photographic silver halide emulsions. Still another object is to provide photographic silver halide emulsions containing non-diffusing sensitizing dyes, which do not cause staining on development of the latent image. Still another object is to provide new merocyanine dyes which are useful in sensitizing the aforesaid photographic silver halide emulsions. Another object is to provide methods for making these new sensitizing dyes. Other objects will become apparent from a consideration of the following description and examples.

According to our invention, we accomplish the above objects by incorporating a merocyanine dye containing a 2-alkylthio-5(4)-thiazolone nucleus in photographic silver halide emulsions.

The merocyanine dyes containing a 2-alkyl-thio-5(4)-thiazolone nucleus which can advantageously be used in our invention can be represented by the following general formula:



sents a positive integer of from 1 to 20), L represents a methine group (e. g.  $=\text{CH}-$ ,  $=\text{CR}'-$ , wherein R' represents an alkyl group, such as methyl, ethyl, etc.), n represents a positive integer from 1 to 2, d represents a positive integer from 1 to 3, and Z represents the non-metallic atoms necessary to complete a heterocyclic nucleus containing from 5 to 6 atoms in the heterocyclic ring, such as a heterocyclic nucleus selected from the group consisting of those of the thiazole series (e. g. thiazole, 4-methylthiazole, 4-phenylthiazole, 5-methylthiazole, 5-phenylthiazole, 4,5-dimethylthiazole, 4,5-diphenylthiazole, 4-(2-thienyl)thiazole, etc.), those of the benzothiazole series (e. g. benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dioxymethylenebenzothiazole, 5-hydroxybenzothiazole, 6-hydroxybenzothiazole, etc.), those of the naphthothiazole series (e. g.  $\alpha$ -naphthothiazole,  $\beta$ -naphthothiazole, 5-methoxy- $\beta$ -naphthothiazole, 5-ethoxy- $\beta$ -naphthothiazole, 8-methoxy- $\alpha$ -naphthothiazole, 7-methoxy- $\alpha$ -naphthothiazole, etc.), those of the thionaphtheno-7',6',4,5-thiazole series (e. g. 4'methoxythionaphtheno-7',6',4,5-thiazole, etc.), those of the oxazole series (e. g. 4-methyloxazole, 5-methyloxazole, 4-phenyloxazole, 4,5-diphenyloxazole, 4-ethyloxazole, 4,5-dimethyloxazole, 5-phenyloxazole, etc.), those of the benzoxazole series (e. g. benzoxazole, 5-chlorobenzoxazole, 5-methylbenzoxazole, 5-phenyloxazole, 6-methylbenzoxazole, 5,6-dimethylbenzoxazole, 4,5-dimethylbenzoxazole, 5-methoxybenzoxazole, 5-ethoxybenzoxazole, 5-chlorobenzoxazole, 6-methoxybenzoxazole, 5-hydroxybenzoxazole, 6-hydroxybenzoxazole, etc.), those of the naphthoxazole series (e. g.  $\alpha$ -naphthoxazole,  $\beta$ -naphthoxazole, etc.), those of the selenazole series (e. g. 4-methylselenazole, 4-phenylselenazole, etc.), those of the benzosele-nazole series (e. g. benzosele-nazole, 5-chlorobenzosele-nazole, 5-methoxybenzosele-nazole, 5-hydroxybenzosele-nazole, tetrahydrobenzosele-nazole, etc.), those of the naphthosele-nazole series (e. g.  $\alpha$ -naphthosele-nazole,  $\beta$ -naphthosele-nazole, etc.), those of the thiazoline series (e. g. thiazoline, 4-methylthiazoline, etc.), those of the 2-quinoline

series (e. g. quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline, etc.), those of the 4-quinoline series (e. g. quinoline, 6-methoxyquinoline, 7-methylquinoline, 8-methylquinoline, etc.), those of the 1-isoquinoline series (e. g. isoquinoline, 3,4-dihydroisoquinoline, etc.), those of the 3-isoquinoline series (e. g. isoquinoline, etc.), those of the 3,3-dimethylindolenine series (e. g. 3,3-dimethylindolenine, 3,3,5-trimethylindolenine, 3,3,7-trimethylindolenine, etc.), the pyridine series (e. g. pyridine, 5-methylpyridine, etc.), etc. Merocyanine dyes wherein  $R_1$  in the above formula represents an alkyl group of the formula  $C_qH_{2q+1}$  wherein  $q$  represents a positive integer from 6 to 20 have been found to be particularly useful in practicing our invention in that they are substantially non-diffusing when incorporated in a photographic silver halide emulsion and do not give rise to stain upon development of the latent image.

The dyes of Formula I above wherein  $d$  represents 1 can advantageously be prepared by condensing a compound selected from those represented by the following general formula:



wherein R<sub>1</sub> has the values set forth above, with a cyclammonium quaternary salt selected from those represented by the following general formula:



wherein R, n, and Z have the values set forth above, Y represents an electronegative group, such as chlorine, bromine, alkoxy (e. g. methoxyl, ethoxyl, etc.), or a  $-\text{S}-\text{R}_2$  group wherein  $\text{R}_2$  represents an alkyl group, such as methyl, ethyl, etc., or an aryl group, such as phenyl, o-, m-, and p-tolyl, etc., and X represents an anion, such as chloride, bromide, iodide, perchlorate, thiocyanate, sulfonate, methylsulfate, ethylsulfate, benzenesulfonate, p-toluenesulfonate, acetate, etc.

The dyes of Formula I above wherein  $d$  represents 2 or 3 can advantageously be prepared by condensing a compound selected from those represented by Formula II above with a cyclammonium quaternary salt selected from those represented by the following general formula:



wherein R, L, n, and Z have the values set forth above,  $R_3$  represents the acyl group of a carboxylic acid, such as acetyl, propionyl, benzoyl, etc. (especially an acyl group of an aliphatic carboxylic acid),  $R_4$  represents a hydrogen atom or an aryl group, such as phenyl, o-, m-, and p-tolyl, etc.,  $p$  represents a positive integer from 1 to 2, and  $X_1$  represents an anion, such as those set forth above for X, for example.

Each of the above-mentioned condensations is advantageously carried out in the presence of an acid-binding agent, such as the trialkylamines (e. g. triethylamine, tri-*n*-propylamine, triisopropylamine, tri-*n*-butylamine, tri-*n*-amylamine, etc.), *N,N*-dialkylanilines (e. g. *N,N*-dimethyl-aniline, *N,N*-diethyl-aniline, etc.), *N*-alkylpiper-

idines (e. g. N-methylpiperidine, n-ethylpiperidine, etc.), heterocyclic amines (e. g. pyridine, quinoline, etc.), etc.

Inert solvents can also be present during the condensations, if desired. Typical solvents include the lower aliphatic alcohols, such as ethanol, n-propanol, isopropanol, n-butanol, etc., diethyl ether, acetone, 1,4-dioxane, n-pentane, n-heptane, benzene, toluene, chloroform, carbon-tetrachloride, etc. Heat accelerates the condensations, and temperatures varying from room temperature (about 25° C.) to the reflux temperature of the reaction mixture can advantageously be employed.

15 The intermediates represented by Formula II above can advantageously be prepared by refluxing an ester selected from those represented by the following general formula:



wherein  $R_1$  has the values set forth above with acetic anhydride. The intermediates represented by Formula II can advantageously be prepared by intermixing an aqueous alkali metal hydroxide solution, carbon disulfide, and glycine, followed by addition of an alkyl halide to the alkali metal salt



formed, heating the mixture at a temperature of from about 40 to 100° C., and acidifying the reaction mixture to give the desired ester represented by Formula V above. These steps can be illustrated by the following general equations:



wherein M represents an alkali metal and X<sub>2</sub> represents a halogen atom. This method has been previously described by Cook, Harris, Heilbron, and Shaw—"Jour. Chem. Soc." (London) 1948, pp. 1056-1060.

pp. 1030-1031.

Alternatively, the merocyanine dyes of Formula I above where  $d$  represents 2 (i. e. dimethine merocyanine dyes) can advantageously be prepared by condensing a compound selected from those represented by the following general formula:



wherein  $R_1$  has the values set forth above and  $R_5$  represents a hydrogen atom or an alkyl group (e. g. methyl, ethyl, etc. groups), with a cyclammonium quaternary salt selected from those represented by the following general formula:



wherein R, X, n, and Z have the values set forth above. These condensations can advantageously be carried out in the presence of an acid-

binding agent, such as the trialkylamines (e. g. triethylamine, tri-n-propylamine, triisopropylamine, tri-n-butylamine, tri-n-amylamine, etc.), N,N-dialkylanilines (e. g. N,N-dimethylaniline, N,N-diethylaniline, etc.), N-alkylpiperidines (e. g. N-methylpiperidines, N-ethylpiperidines, etc.), heterocyclic amines (e. g. pyridine, quinoline, etc.), etc. An inert solvent can also be employed, if desired. Typical solvents include the lower aliphatic alcohols (e. g. methanol, ethanol, n-propanol, isopropanol, n-butanol, etc.), diethyl ether, 1,4-dioxane, n-pentane, n-hexane, benzene, toluene, chloroform, carbontetrachloride, etc. Heating accelerates the condensations, and temperatures varying from room temperature (about 25° C.) to the reflux temperature of the reaction mixture can advantageously be used.

The intermediates represented by Formula VI above can advantageously be prepared by heating together a mixture of one of the esters represented by Formula V above, acetic anhydride, and an ortho ethyl ester selected from those represented by the following general formula:



wherein  $R_5$  has the values set forth above. Temperatures of from 100 to 150° C. can advantageously be used to accelerate the condensations.

The following examples illustrate further the manner whereby we practice our invention.

*Example 1.*—[2-(3-ethylbenzoxazole)] [4-(2-ethylthio-5(4)-thiazolone)] dimethinemero-cyanine



2-ethylthio-4-ethoxymethylene-5(4)-thiazolone was obtained by heating 9.0 g. of N-dithiocarbethoxyglycine on a steam bath along with 40 cc. of acetic anhydride and 12 cc. of ethyl orthoformate for 30 minutes and then distilling off liquid until an oil remained. The resultant oil was then refluxed for 5 minutes with 14.5 g. of 2-methylbenzoxazole ethiodide, 40 cc. of ethanol, and 10 cc. of triethylamine, and the reaction mixture then chilled. The dye was recrystallized from ethanol as flat, steel-blue needles melting at 156° C. It sensitized a gelatino silver chloride emulsion strongly with a maximum at 530 m $\mu$  and a gelatino silver bromide emulsion with a maximum at 540 m $\mu$ .

*Example 2.*—[2-(1-ethylquinoline)] [4-(2-ethylthio-5(4)-thiazolone)] dimethinemero-cyanine



4.44 g. of 2- $\beta$ -acetanilidovinylquinoline ethiodide, 2-ethylthio-5(4)-thiazolone (obtained by heating 1.8 g. of N-dithiocarbethoxyglycine with acetic anhydride and driving off the residual liquids), 25 cc. of ethanol, and 2 cc. of triethylamine were refluxed for 5 minutes and the reaction mixture then chilled. The desired dye was obtained as soft, dark green needles melting at 163° C. on recrystallization from a benzene-ethanol mixture. It sensitized a gelatino silver chlo-

ride emulsion with a flat maximum lying between 530 and 590 m $\mu$ .

*Example 3.*—[2-(3-ethylbenzoxazole)] [4-(2-ethylthio-5(4)-thiazolone)] dimethinemero-cyanine



This dye was prepared in the same manner as the dye of Example 1 by replacing the 2-methylbenzoxazole ethiodide used in that example by a molecularly equivalent amount of 2-methylbenzoxazole ethiodide. The desired dye was obtained as blue-grey prisms melting at 184° C. on recrystallization from benzene. It sensitized a gelatino silver bromide emulsion strongly.

*Example 4.*—[2-(3-methylthiazoline)] [4-2-ethylthio-5(4)-thiazolone] dimethinemero-cyanine



This dye was prepared in the same manner as the dye of Example 1 by replacing the quaternary salt used in that example by a molecularly equivalent amount of 2-methylthiazoline methiodide. The desired dye was obtained as maroon needles melting at 129° C. on recrystallization from ethanol. It sensitized a gelatino silver chloride emulsion with a maximum at 500 m $\mu$  and a gelatino silver bromide emulsion with a maximum at 530 m $\mu$ .

*Example 5.*—[2-(3-ethyl-4-methylthiazole)] [4-(2-ethylthio-5(4)-thiazolone)] dimethinemero-cyanine



This dye was prepared in the same manner as the dye of Example 1 by replacing the 2-methylbenzoxazole ethiodide used in that example by a molecularly equivalent amount of 2,4-dimethylthiazole ethiodide. The desired dye was obtained as green prisms melting at 154° C. on recrystallization from a benzene-ethanol mixture. It sensitized a gelatino silver bromide emulsion strongly.

*Example 6.*—[4-(1-ethylquinoline)] [4-(2-ethylthio-5(4)-thiazolone)] dimethinemero-cyanine



This dye was prepared in the same manner as the dye of Example 1 by replacing the 2-methylbenzoxazole ethiodide used in that example by a molecularly equivalent amount of lepidinium ethiodide. The desired dye was obtained as blue plates melting at 143° C. on recrystallization from ethanol. It sensitized a gelatino silver chloride emulsion with a maximum at 510 m $\mu$  and

a gelatino silver bromide emulsion with a flat maximum lying between 560 and 640 m $\mu$ .

Example 7.—[2-(3-ethylbenzothiazole) 1 [4-(2-ethylthio-5(4)-thiazolone)] dimethinememerocyanine



This dye was prepared in the same manner as the dye of Example 2 by replacing the quaternary salt used in that example by a molecularly equivalent amount of 2- $\beta$ -acetanilidovinylbenzothiazole ethiodide. The desired dye was obtained as blue-grey prisms melting at 173° C. on recrystallization from benzene. It sensitized a gelatino silver chloride emulsion with a maximum at 550 m $\mu$  and a gelatino silver bromide emulsion with a maximum at 580 m $\mu$ .

Example 8.—[2-(3-ethyl-4-p-tolylthiazole) 1 [4-(2-ethylthio-5(4)-thiazolone)] dimethinememerocyanine



This dye was prepared in the same manner as the dye of Example 1 by replacing the quaternary salt used in that example by a molecularly equivalent amount of 2-methyl-4-p-tolylthiazole ethiodide. The desired dye was obtained as steel blue crystals melting at 182° C. on recrystallization from benzene. It sensitized a gelatino silver chloride emulsion with a flat maximum lying between 490 and 550 m $\mu$ , and a gelatino silver bromide emulsion with a flat maximum lying between 530 and 560 m $\mu$ .

Example 9.—[2-(1-ethyl- $\beta$ -naphthothiazole) 1 [4-(2-ethylthio-5(4)-thiazolone)] dimethinememerocyanine



The dye was prepared in the same manner as the dye of Example 2 by replacing the quaternary salt used in that example by a molecularly equivalent amount of 2- $\beta$ -acetanilidovinyl- $\beta$ -naphthothiazole ethiodide. The desired dye was obtained as flat maroon needles melting at 172° C. on recrystallization from benzene. It sensitized a gelatino silver chloride emulsion with a maximum at 560 m $\mu$ .

Example 10.—[2-(3-ethylbenzoxazole) 1 [4-(2-ethylthio-5(4)-thiazolone)] -  $\beta$ -methyldimethinememerocyanine



1.8 g. of N-dithiocarbethoxyglycine, 15 cc. of acetic anhydride, and 5 cc. of ethyl orthoacetate were heated on a steam bath for one hour, and the liquids removed under a vacuum. To the residual oil were added 2.9 g. of 2-methylbenzoxazole ethiodide, 10 cc. of ethanol, and 2 cc. of triethylamine, and the whole was refluxed for 15 minutes and then chilled. The precipitate obtained was filtered off and recrystallized from benzene as fine, rust-colored needles melting at 118° C. It sensitized a gelatino silver chloride emulsion with a maximum at 516 m $\mu$  and a gelatino silver bromide emulsion with a maximum at 540 m $\mu$ .

Example 11.—[2-(3-ethylbenzothiazole) 1 [4-(2-ethylthio-5(4)-thiazolone)] -  $\beta$ -methyldimethinememerocyanine



This dye was obtained in the same manner as the dye of Example 10 by replacing the quaternary salt used in that example by a molecularly equivalent amount of 2-methylbenzothiazole ethiodide. The desired dye was obtained as fine purple needles melting at 130° C. on recrystallization from benzene. It sensitized a gelatino silver chloride emulsion with a maximum at 550 m $\mu$  and a gelatino silver bromide emulsion with a maximum at 570 m $\mu$ .

Example 12.—[2-(3-ethylbenzoselenazole) 1 [4-(2-ethylthio-5(4)-thiazolone)] -  $\beta$ -methyldimethinememerocyanine



This dye was prepared in the same manner as the dye of Example 10 by replacing the quaternary salt used in that example by a molecularly equivalent amount of 2-methylbenzoselenazole ethiodide. The desired dye was obtained as steel blue prisms melting at 140° C. on recrystallization from benzene. It sensitized a gelatino silver chloride emulsion with a maximum at 560 m $\mu$  and a gelatino silver bromide emulsion with a maximum at 570 m $\mu$ .

Example 13.—[2-(3-methylthiazoline) 1 [4-(2-ethylthio-5(4)-thiazolone)] -  $\beta$ -methyldimethinememerocyanine



This dye was prepared in the same manner as the dye of Example 10 by replacing the quaternary salt used in that example by a molecularly equivalent amount of 2-methylthiazoline methiodide. The desired dye was obtained as grey-red needles melting at 133° C. on recrystallization from a benzene-petroleum ether mixture. It sensitized a gelatino silver chloride emulsion with a maximum at 500 m $\mu$ .

Example 14.—[2-(1-ethylquinoline)] [4-(2-ethylthio-5(4)-thiazolone)]- $\beta$ -methyldimethinemerocyanine



This dye was prepared in the same manner as the dye of Example 10 by replacing the quaternary salt used in that example by a molecularly equivalent amount of quinaldinium ethiodide. The desired dye was obtained as fine green needles on recrystallization from benzene and had a melting point of 130° C. It sensitized a gelatino silver chloride emulsion with a maximum at 580 m $\mu$ . 10

Example 15.—[2-(3-ethyl-4-methylthiazole)] [4-(2-ethylthio-5(4)-thiazolone)]- $\beta$ -methyldimethinemerocyanine



This dye was prepared in the same manner as the dye of Example 10 by replacing the quaternary salt used in that example by a molecularly equivalent amount of 2,4-dimethylthiazole ethiodide. The desired dye was obtained as glossy red needles melting at 154° C. on recrystallization from a benzene-petroleum ether mixture. It sensitized both a gelatino silver chloride emulsion and a gelatino silver bromide emulsion with a maximum at 530 m $\mu$ . 15

Example 16.—[2-(1-ethylquinoline)] [4-(2-benzylthio-5(4)-thiazolone)] dimethinemerocyanine



This dye was prepared in the same manner as the dye of Example 1 by replacing the quaternary salt used in that example by a molecularly equivalent amount of quinaldinium ethiodide and the 4-ethoxymethylene intermediate by a molecularly equivalent amount of 2-benzylthio-4-ethoxymethylene-5(4)-thiazolone. The desired dye was obtained as green needles melting at 207° C. on recrystallization from ethanol. It sensitized a gelatino silver chloride emulsion with a flat maximum lying between 550 and 580 m $\mu$  and a gelatino silver bromide emulsion with a flat maximum lying between 550 and 560 m $\mu$ . 20

Example 17.—[2-(3-ethylbenzothiazole)] [4-(2-benzylthio-5(4)-thiazolone)] dimethinemerocyanine



This dye was obtained in the same manner as the dye of Example 1 by replacing the quaternary salt used in that example by a molecularly equivalent amount of 2-methylbenzothiazole ethiodide and the 4-ethoxymethylene intermediate by a mo- 25

lecularly equivalent amount of 2-benzylthio-4-ethoxymethylene-5(4)-thiazolone. The desired dye was obtained as red needles melting at 179° C. on recrystallization from ethanol. It sensitized a gelatino silver chloride emulsion with a maximum at 550 m $\mu$ .

Example 18.—[2-(3-ethylbenzoselenazole)] [4-(2-benzylthio-5(4)-thiazolone)] dimethinemerocyanine



This dye was obtained in the same manner as the dye of Example 1 by replacing the quaternary salt used in that example by a molecularly equivalent amount of 2-methylbenzoselenazole ethiodide and the 4-ethoxymethylene intermediate by a molecularly equivalent amount of 2-benzylthio-4-ethoxymethylene-5(4)-thiazolone. The desired dye was obtained as violet needles melting at 165° C. or recrystallization from ethanol. It sensitized a gelatino silver chloride emulsion with a maximum at 560 m $\mu$ . 25

Example 19.—[2-(3-ethylbenzoxazole)] [4-(2-benzylthio-5(4)-thiazolone)] dimethinemerocyanine



This dye was prepared in the same manner as the dye of Example 1 by replacing the 4-ethoxymethylene intermediate used in that example by a molecularly equivalent amount of 2-benzylthio-4-ethoxymethylene-5(4)-thiazolone. The desired dye melted at 193° C. on recrystallization from ethanol and sensitized a gelatino silver chloride emulsion with a maximum at 510 m $\mu$ . 30

Example 20.—[2-(1-ethylpyridine)] [4-(2-benzylthio-5(4)-thiazolone)] dimethinemerocyanine



This dye was prepared in the same manner as the dye of Example 1 by replacing the quaternary salt used in that example by a molecularly equivalent amount of  $\alpha$ -picoline ethiodide and the 4-ethoxymethylene intermediate by a molecularly equivalent amount of 2-benzylthio-4-ethoxymethylene-5(4)-thiazolone. The desired dye was obtained as purple needles melting at 152° C. on recrystallization from ethanol. It sensitized a gelatino silver chloride emulsion with a flat maximum lying between 490 and 530 m $\mu$  and a gelatino silver bromide emulsion with a maximum at 530 m $\mu$ . 55

Example 21.—[4-(1-ethylquinoline)] [4-(2-benzylthio-5(4)-thiazolone)] dimethinemerocyanine



11

This dye was obtained in the same manner as the dye of Example 1 by replacing the quaternary salt used in that example by a molecularly equivalent amount of lepidinium ethiodide and the 4-ethoxymethylene intermediate by a molecularly equivalent amount of 2-benzylthio-4-ethoxymethylene-5(4)-thiazolone. The desired dye was obtained as blue needles melting at 162° C. on recrystallization from ethanol. It sensitized a gelatino silver bromide emulsion with maxima at 10 680 and 730 m $\mu$ .

Example 22.—[2-(3-methylthiazoline) ] [4-(2-benzylthio-5(4)-thiazolone) ] dimethinemero-cyanine.



This dye was prepared in the same manner as the dye of Example 1 by replacing the quaternary salt used in that example by a molecularly equivalent amount of 2-methylthiazoline methiodide and the 4-ethoxymethylene intermediate by a molecularly equivalent amount of 2-benzylthio-4-ethoxymethylene-5(4)-thiazolone. The desired dye was obtained as red-green prisms melting at 171° C. on recrystallization from a benzene-ethanol mixture. It sensitized a gelatino silver chloride emulsion with a maximum at 500 m $\mu$  and a gelatino silver bromide emulsion with a maximum at 525 m $\mu$ .

This dye was prepared in the same manner as the dye of Example 1 by replacing the quaternary salt used in that example by a molecularly equivalent amount of 2-methylthiazoline methiodide and the 4-ethoxymethylene intermediate by a molecularly equivalent amount of 2-benzylthio-4-ethoxymethylene-5(4)-thiazolone. The desired dye was obtained as red-green prisms melting at 171° C. on recrystallization from a benzene-ethanol mixture. It sensitized a gelatino silver chloride emulsion with a maximum at 500 m $\mu$  and a gelatino silver bromide emulsion with a maximum at 525 m $\mu$ .

Example 23.—[2-(1-ethyl- $\beta$ -naphthothiazole) ] [4-(2-benzylthio-5(4)-thiazolone) ] dimethinemero-cyanine



This dye was prepared in the same manner as the dye of Example 1 by replacing the quaternary salt used in that example by a molecularly equivalent amount of 2-methyl- $\beta$ -naphthothiazole ethiodide and the 4-ethoxymethylene intermediate by a molecularly equivalent amount of 2-benzylthio-4-ethoxymethylene-5(4)-thiazolone. The desired dye was obtained as purple needles melting at 215° C. on recrystallization from a benzene-ethanol mixture. It sensitized a gelatino silver chloride emulsion with a maximum at 570 m $\mu$  and a gelatino silver bromide emulsion with a maximum at 580 m $\mu$ .

12

Example 24.—[4-(1-methylpyridine) ] [4-(2-benzylthio-5(4)-thiazolone) ] dimethinemero-cyanine



This dye was prepared in the same manner as the dye of Example 1 by replacing the quaternary salt used in that example by a molecularly equivalent amount of  $\gamma$ -picoline methiodide and the 4-ethoxymethylene intermediate by a molecularly equivalent amount of 2-benzylthio-4-ethoxymethylene-5(4)-thiazolone. The desired dye was obtained as green crystals melting at 172° C. on recrystallization from ethanol. It sensitized a gelatino silver chloride emulsion with a flat maximum lying between 540 and 560 m $\mu$ .

Example 25.—[2-(3-methylthiazoline) ] [4-(2-n-octylthio-5(4)-thiazolone) ] dimethinemero-cyanine



1.4 g. of N-dithiocarbo-n-octoxyglycine, 10 cc. of acetic anhydride, and 5 cc. of ethyl orthoformate were heated together on an oil bath at 130° C. for 30 minutes, and the volatile liquids removed under a vacuum. To the residual brown oil were added 1.3 g. of 2-methylthiazoline methiodide, 10 cc. of ethanol, and 2 cc. of triethylamine, and the whole heated on a steam bath for 5 minutes. After chilling overnight, brown crystals weighing 0.8 g. were collected, washed with ethanol and twice recrystallized from this alcohol as small purple needles melting at 81° C. It sensitized a gelatino silver chloride emulsion with a maximum at 500 m $\mu$  and a gelatino silver bromide emulsion with a maximum at 520 m $\mu$ .

Example 26.—[2-(3-ethylthiazoline) ] [4-(2-n-octylthio-5(4)-thiazolone) ] dimethinemero-cyanine



This dye was obtained in the same manner as the dye of Example 25 by replacing the quaternary salt used in that example by 1.35 g. of 2-methylthiazoline ethiodide. It was obtained as fine orange crystals melting at 86° C. on recrystallization from ethanol. It sensitized a gelatino silver chloride emulsion with a maximum at 500 m $\mu$  a gelatino silver bromide emulsion with a maximum at 520 m $\mu$ .

Example 27.—[2-(3-ethylbenzoxazole) ] [4-(2-n-octylthio-5(4)-thiazolone) ] dimethinemero-cyanine



This dye was obtained in the same manner as the dye of Example 25 by replacing the quater-

## 13

inary salt used in that example by 1.45 g. of 2-methylbenzoxazole ethiodide. It was obtained as glittering orange plates melting at 130° C. on recrystallization from methanol. It sensitized a gelatino silver chloride emulsion with a maximum at 530 m $\mu$  and a gelatino silver bromide emulsion with a maximum at 540 m $\mu$ .

*Example 28.—[2 - (5 - chloro-3-ethylbenzothiazole) ] [4-(2 - n - octylthio - 5(4) - thiazolone) ] dimethinemero-cyanine*



This dye was obtained in the same manner as the dye of Example 25 by replacing the quaternary salt used in that example by 1.95 g. of 5-chloro-2-methylbenzothiazole etho-p-toluenesulfonate. It formed purple needles melting at 156° C. on recrystallization from benzene. It sensitized a gelatino silver chloride emulsion with a maximum at 560 m $\mu$  and a gelatino silver bromide emulsion with a maximum at 580 m $\mu$ .

*Example 29.—[2 - (3-ethylbenzothiazole) ] [4-(2-n-octylthio - 5(4) - thiazolone) ] dimethinemero-cyanine*



This dye was obtained in the same manner as the dye of Example 25 by replacing the quaternary salt used in that example by 1.55 g. of 2-methylbenzothiazole ethiodide. It was obtained as dark red needles melting at 81° C. from a benzene-methanol mixture. It sensitized a gelatino silver chloride emulsion with a maximum at 550 m $\mu$  and a gelatino silver bromide emulsion with a maximum at 580 m $\mu$ .

*Example 30.—[2-(3-ethylbenzoselenazole) ] [4-(2-n-octylthio-5(4)-thiazolone) ] dimethinemero-cyanine*



This dye was obtained in the same manner as the dye of Example 25 by replacing the quaternary salt used in that example by 1.75 g. of 2-methylbenzoselenazole ethiodide. It formed glossy, flat, violet needles melting at 86° C. from a benzene-methanol mixture. It sensitized a gelatino silver chloride emulsion with a maximum at 570 m $\mu$  and a gelatino silver bromide emulsion with a maximum at 590 m $\mu$ .

*Example 31.—[2-(3-ethylthiazoline) ] [4-(2-ethylthio-5(4)-thiazolone) ] dimethinemero-cyanine*



## 14

This dye was prepared in the same manner as the dye of Example 1 by replacing the quaternary salt used in that example by a molecularly equivalent amount of 2-methylthiazoline ethiodide. The desired dye was obtained as yellow plates melting at 121° C. on recrystallization from ethanol. It sensitized a gelatino silver chloride emulsion with a maximum at 500 m $\mu$  and a gelatino silver bromide emulsion with a maximum at 525 m $\mu$ .

*Example 32.—[2-(3-ethylbenzoxazole) ] [4-(2-n-dodecylthio-5(4)-thiazolone) ] dimethinemero-cyanine*



This dye was prepared in the same manner as the dye of Example 1 by replacing the N-dithiocarbethoxyglycine used in that example by a molecularly equivalent amount of N-dithiocarbo-n-dodecoxyglycine. The desired dye was obtained as a rust-colored powder melting at 103° C. on recrystallization from methanol. It sensitized a gelatino silver chloride emulsion with a maximum at 510 m $\mu$  and a gelatino silver bromide emulsion with a maximum at 530 m $\mu$ .

*Example 33.—[2-(3-ethylbenzoxazole) ] [4-(2-n-hexylthio - 5(4) - thiazolone) ] dimethinemero-cyanine*



This dye was prepared in the same manner as the dye of Example 1 by replacing the N-dithiocarbethoxyglycine used in that example by a molecularly equivalent amount of N-dithiocarbo-n-hexoglycine. The desired dye was obtained as glossy, rust-colored plates melting at 143° C. on recrystallization from ethanol. It sensitized a gelatino silver chloride emulsion with a maximum at 500 m $\mu$  and a gelatino silver bromide emulsion with a maximum at 530 m $\mu$ .

*Example 34.—[2-(3-ethylbenzoxazole) ] [4-(2-n-heptylthio - 5(4) - thiazolone) ] dimethinemero-cyanine*



This dye was prepared in the same manner as the dye of Example 1 by replacing the N-dithiocarbethoxyglycine used in that example by a molecularly equivalent amount of N-dithiocarbo-n-heptoxyglycine. The desired dye was obtained as glossy, rust-colored plates melting at 133° C. on recrystallization from ethanol. It sensitized a gelatino silver chloride emulsion with a maximum at 500 m $\mu$  and a gelatino silver bromide emulsion with a maximum at 530 m $\mu$ .

15

Example 35.—[2-(3-ethylbenzoxazole)] [4-(2- $\gamma$ -phenylpropylthio-5(4)-thiazolone)] dimethinemerocyanine



This dye was prepared in the same manner as the dye of Example 1 by replacing the N-dithiocarbethoxyglycine used in that example by a molecularly equivalent amount of N-dithiocarbonyl- $\gamma$ -phenylpropoxyglycine. The desired dye was obtained as red crystals melting at 170° C. on recrystallization from ethanol. It sensitized a gelatino silver chloride emulsion with a maximum at 500 m $\mu$  and a gelatino silver bromide emulsion with a maximum at 530 m $\mu$ .

Example 36.—[2-(1-ethyl- $\beta$ -naphthothiazole)] [4-(2-ethylthio-5(4)-thiazolone)]  $\beta$ -methyl-dimethinemerocyanine



This dye was prepared in the same manner as the dye of Example 10 by replacing the quaternary salt used in that example by a molecularly equivalent amount of 2-methyl- $\beta$ -naphthothiazole ethiodide. The desired dye was obtained as mauve needles melting at 209° C. on recrystallization from benzene. It sensitized a gelatino silver chloride emulsion with a maximum at 550 m $\mu$  and a gelatino silver bromide emulsion with a maximum at 575 m $\mu$ .

Example 37.—[2-(3-ethylbenzoxazole)] [4-(2-n-decylthio-5(4)-thiazolone)] dimethinemerocyanine



This dye was prepared in the same manner as the dye of Example 1 by replacing the N-dithiocarbethoxyglycine used in that example by a molecularly equivalent amount of N-dithiocarbonyl-decoxyglycine. The desired dye was obtained as an orange powder melting at 106° C. on recrystallization from ethanol. It sensitized a gelatino silver chloride emulsion with a maximum at 510 m $\mu$  and a gelatino silver bromide emulsion with a maximum at 530 m $\mu$ .

Example 38.—[2-(3-ethylbenzoxazole)] [4-(2-n-decylthio-5(4)-thiazolone)]  $\beta$ -methyl-dimethinemerocyanine



This dye was prepared in the same manner as the dye of Example 10 by replacing the N-dithio-

16

carbethoxyglycine used in that example by a molecularly equivalent amount of N-dithiocarbonyl-decoxyglycine. The desired dye was obtained as soft, orange needles melting at 68° C. on recrystallization from ethanol. It sensitized a gelatino silver chloride emulsion with a maximum at 510 m $\mu$  and a gelatino silver bromide emulsion with a maximum at 530 m $\mu$ .

Example 39.—[2-(3-ethylbenzoxazole)] [4-(2-n-decylthio-5(4)-thiazolone)]  $\beta$ -ethyl-dimethinemerocyanine



This dye was prepared in the same manner as the dye of Example 10 by replacing the ethyl orthoacetate used in that example by a molecularly equivalent amount of ethyl orthopropionate and the N-dithiocarbethoxyglycine by a molecularly equivalent amount of N-dithiocarbonyl-decoxyglycine. The desired dye was obtained as orange needles melting at 96° C. on recrystallization from ethanol. It sensitized a gelatino silver chloride emulsion with a maximum at 510 m $\mu$  and a gelatino silver bromide emulsion with a maximum at 530 m $\mu$ .

Example 40.—[2-(3-ethylbenzosenazole)] [4-(2-n-heptylthio-5(4)-thiazolone)] dimethinemerocyanine



This dye was prepared in the same manner as the dye of Example 1 by replacing the quaternary salt used in that example by a molecularly equivalent amount of 2-methylbenzosenazole ethiodide, and the N-dithiocarbethoxyglycine by a molecularly equivalent amount of N-dithiocarbonyl-heptoxyglycine. The desired dye was obtained as glossy, violet needles melting at 112° C. on recrystallization from ethanol. It sensitized a gelatino silver chloride emulsion with a maximum at 560 m $\mu$  and a gelatino silver bromide emulsion with a maximum at 585 m $\mu$ .

Example 41.—[2-(3-ethylbenzothiazole)] [4-(2-ethylthio-5(4)-thiazolone)] tetramethinemerocyanine



This dye was prepared in the same manner as the dye of Example 2 by replacing the quaternary salt used in that example by a molecularly equivalent amount of 2- $\alpha$ -acetanilido-1,4-butadienylbenzothiazole ethiodide. The desired dye was obtained as a blue crystalline powder melting at 179° C. on recrystallization from ethanol. It strongly sensitized a gelatino silver bromide emulsion.

In a like manner, by replacing the quaternary salt used in Example 2 by a molecularly equivalent amount of 2-methylthiobenzothiazole ethio-

17

dide [2-(3-ethylbenzothiazole)] [4-(2-ethylthio-5(4)-thiazolone)]merocyanine represented by the following general formula:



can be obtained.

The N-dithiocarbo-n-octoxyglycine employed in Example 25 above was prepared as follows:

*Example 42.* — *N* - dithiocarbo - *n* - octoxyglycine



22.4 g. of potassium hydroxide were dissolved in 50 cc. of water and the solution chilled. There were then added 15.0 g. of glycine and 15.2 g. of carbondisulfide, and the whole shaken mechanically until a clear orange solution resulted. A solution of 38.6 g. of n-octylbromide in 50 cc. of ethanol was added, and the mixture heated for 30 minutes on a steam bath. To the resulting one-phase solution there were added 100 cc. of water, and the cloudiness resulting removed by extraction with diethyl ether. The aqueous layer was warmed gently under reduced pressure to expel any dissolved ether, the solution chilled, and acidified with concentrated hydrochloric acid. The precipitate was collected on a filter, washed with water, air-dried, and recrystallized from petroleum ether (E. P. 60-80° C.) as glistening plates melting at 100° C.

By replacing the n-octylbromide used in the above example by molecularly equivalent amounts of n-hexyl, n-heptyl, n-decyl, n-dodecyl, and  $\gamma$ -phenylpropyl halide, respectively, the following n-dithiocarbalkoxyglycines were prepared:

*Example 43.* — *N* - dithiocarbo - *n* - hexoxyglycine



Obtained as soft, glistening plates melting at 95° C. on recrystallization from ligroin.

*Example 44.* — *N* - dithiocarbo - *n* - heptoxyglycine



Obtained as glistening, waxy plates melting at 99° C. on recrystallization from petroleum ether.

*Example 45.* — *N* - dithiocarbo - *n* - decoxyglycine



Obtained as glittering plates melting at 100° C. on recrystallization from a benzene-petroleum ether mixture.

*Example 46.* — *N* - dithiocarbo - *n* - dodecoxyglycine



Obtained as glossy plates melting at 111° C. on recrystallization from ligroin.

*Example 47.* — *N* - dithiocarbo -  $\gamma$  - phenylpropoxyglycine



Obtained as waxy plates melting at 122° C. on recrystallization from a benzene-petroleum ether mixture.

18

To prepare photographic emulsions sensitized with our new dyes, it is only necessary to disperse the dyes in the emulsions. It is convenient to add the dyes to the emulsions from solutions in appropriate solvents. Methyl alcohol has proven satisfactory for this purpose. Ethyl alcohol can also be used. Sensitization by means of these dyes is, of course, directed primarily to the ordinarily employed gelatino-silver-halide developing-out emulsions. The dyes (one or more) are ordinarily incorporated in the washed, finished emulsions and should, of course, be uniformly distributed throughout the emulsion. The concentration of the dyes in the emulsions can vary widely, i. e., from about 5 to about 100 mg. per liter of flowable emulsion. The concentration of the dye will vary according to the type of light-sensitive material in the emulsion and according to the effect desired. The suitable and most economical concentration for any given emulsion will be apparent to those skilled in the art of emulsion making. To prepare a gelatino-silver-halide emulsion sensitized with one more of these dyes, the following procedure is satisfactory. A quantity of the dye is dissolved in methyl alcohol or other suitable solvent, and a volume of this solution (which may be diluted with water) containing from 5 to 100 mg. of dye is slowly added to 1000 cc. of gelatino-silver-halide emulsion, with stirring. Stirring is continued until the dye is uniformly distributed throughout the emulsion. With most of these sensitizing dyes, 10 to 20 mg. of dye per liter of emulsion suffices to produce the maximum sensitizing effect with the ordinary gelatino-silver-bromide (including bromide) emulsions. With gelatino-silver-chloride emulsions somewhat larger concentrations may be required to produce the optimum sensitizing effect. The above statements are only illustrative and are not to be understood as limiting our invention, as it will be apparent that these dyes can be incorporated by other methods in photographic silver halide emulsions customarily employed in the art. For instance, the dyes may be incorporated by bathing a plate of film upon which an emulsion has been coated in a solution of the dye in an appropriate solvent. Bathing methods, however, are not to be preferred ordinarily.

The accompanying drawing further illustrates our invention. Each figure is a diagrammatic reproduction of a spectrogram showing the sensitivity of a gelatino silver bromide (specifically a silver bromide) emulsion containing one of our alkylthio-5(4)-thiazolone dyes. In Fig. 1, the curve depicts the sensitivity of an ordinary gelatino silver bromide emulsion containing [2-(3-methylthiazoline) 1 [4-(2-ethylthio-5(4)-thiazolone)]dimethinemerocyanine. In Fig. 2, the curve depicts the sensitivity of an ordinary gelatino silver bromide emulsion containing [2-(3-ethylbenzothiazole) 1 [4-(2-ethylthio-5(4)-thiazolone)]dimethinemerocyanine. In Fig. 3, the curve depicts the sensitivity of an ordinary gelatino silver bromide emulsion containing [2-(3-ethylbenzothiazole) 1 [4-(2-ethylthio-5(4)-thiazolone)]dimethinemerocyanine.

The dyes of our invention wherein  $R_1$  represents an alkyl group of the formula  $C_qH_{2q+1}$  wherein  $q$  is a positive integer from 6 to 20 have lower solubility and diffusibility in photographic silver halide emulsions than many of the known sensitizing dyes and are especially valuable, therefore, in sensitizing photographic emulsions employed in color photographic elements where

(relative) non-diffusibility of the sensitizing dyes is required for good color-separation. In some color processes, too, substances are present in the emulsions that tend to dissolve the sensitizing dyes from the silver halide grains. Low solubility of these dyes minimizes this tendency. Typical color photographic processes and typical color photographic elements comprising two or more differentially sensitized photographic silver halide emulsions are described in United States Patent 2,113,329, dated April 5, 1938, in British Patents 500,611 and 500,862; each accepted February 10, 1939, in United States Patent 1,985,344, dated December 25, 1934, in United States Patent 1,956,122, dated April 24, 1934, and in United States Patent 1,517,049, dated November 25, 1924, for example. Another case where our new long-chain alkyl dyes are especially useful is in the sensitization of variable contrast materials, such as described in United States Patent 2,384,598, dated September 11, 1945, United States Patent 2,358,169, dated September 12, 1944, and in United States Patent 2,358,060, dated September 12, 1944.

Emulsions sensitized according to our invention can be coated on the usual supports of paper, cellulose acetate film, glass, polyvinyl resin (acetate, acetal, etc.) film, metal, etc., in the usual manner.

What we claim as our invention and desire secured by Letters Patent of the United States is:

1. A photographic silver halide emulsion sensitized with at least one merocyanine dye selected from those represented by the following general formula:



wherein R and R<sub>1</sub> each represents an alkyl group, L represents a methine group, n represents a positive integer from 1 to 2, d represents a positive integer from 1 to 3, and Z represents the non-metallic atoms necessary to complete a heterocyclic nucleus containing from 5 to 6 atoms in the heterocyclic ring.

2. A photographic silver halide emulsion sensitized with at least one merocyanine dye selected from those represented by the following general formula:



wherein R represents an alkyl group of the formula C<sub>m</sub>H<sub>2m+1</sub> wherein m represents a positive integer from 1 to 8, R<sub>1</sub> represents an alkyl group of the formula C<sub>q</sub>H<sub>2q+1</sub> wherein q represents a positive integer from 1 to 20, L represents a methine group, n represents a positive integer from 1 to 2, d represents a positive integer from 1 to 3, and Z represents the non-metallic atoms necessary to complete a heterocyclic nucleus selected from the group consisting of those of the thiazole series, benzothiazole series, naphthothiazole series, oxazole series, benzoxazole series, naphthoxazole series, selenazole series, benzoselenazole series, naphthoselenazole series, thiazoline series, 2-quinoline series, 4-quinoline series, 1-isoquinoline series, 3-isoquinoline series, pyridine series, and 3,3-dimethylindolenine series.

3. A photographic silver halide emulsion sensitized with at least one merocyanine dye selected

from those represented by the following general formula:



wherein R represents an alkyl group of the formula C<sub>m</sub>H<sub>2m+1</sub> wherein m represents a positive integer from 1 to 8, R<sub>1</sub> represents an alkyl group of the formula C<sub>q</sub>H<sub>2q+1</sub> wherein q represents a positive integer from 6 to 20, L represents a methine group, n represents a positive integer from 1 to 2, d represents a positive integer from 1 to 3, and Z represents the non-metallic atoms necessary to complete a heterocyclic nucleus selected from the group consisting of those of the thiazole series, benzothiazole series, naphthothiazole series, oxazole series, benzoxazole series, naphthoxazole series, selenazole series, benzoselenazole series, naphthoselenazole series, thiazoline series, 2-quinoline series, 4-quinoline series, 1-isoquinoline series, 3-isoquinoline series, pyridine series, and 3,3-dimethylindolenine series.

4. A photographic silver bromide emulsion sensitized with at least one merocyanine dye selected from those represented by the following general formula:



wherein R represents an alkyl group of the formula C<sub>m</sub>H<sub>2m+1</sub> wherein m represents a positive integer from 1 to 8, R<sub>1</sub> represents an alkyl group of the formula C<sub>q</sub>H<sub>2q+1</sub> wherein q represents a positive integer from 6 to 20, L represents a methine group, n represents a positive integer from 1 to 2, d represents a positive integer from 1 to 3, and Z represents the non-metallic atoms necessary to complete a heterocyclic nucleus selected from the group consisting of those of the thiazole series, benzothiazole series, naphthothiazole series, oxazole series, benzoxazole series, naphthoxazole series, selenazole series, benzoselenazole series, naphthoselenazole series, thiazoline series, 2-quinoline series, 4-quinoline series, 1-isoquinoline series, 3-isoquinoline series, pyridine series, and 3,3-dimethylindolenine series.

5. A photographic silver halide emulsion sensitized with at least one merocyanine dye selected from those represented by the following general formula:



wherein R represents a primary alkyl group of the formula C<sub>m</sub>H<sub>2m+1</sub> wherein m represents a positive integer from 1 to 8, R<sub>1</sub> represents a primary alkyl group of the formula C<sub>q</sub>H<sub>2q+1</sub> wherein q represents a positive integer from 1 to 20, L represents a methine group, d represents a positive integer from 1 to 3, and Z represents the non-metallic atoms necessary to complete a heterocyclic nucleus of the benzothiazole series.

6. A photographic silver halide emulsion sensitized with at least one merocyanine dye selected from those represented by the following general formula:



75 wherein R represents a primary alkyl group of

21

the formula  $C_mH_{2m+1}$  wherein  $m$  represents a positive integer from 1 to 8,  $R_1$  represents a primary alkyl group of the formula  $C_qH_{2q+1}$  wherein  $q$  represents a positive integer from 1 to 20,  $L$  represents a methine group,  $d$  represents a positive integer from 1 to 3, and  $Z$  represents the non-metallic atoms necessary to complete a heterocyclic nucleus of the benzoxazole series.

7. A photographic silver halide emulsion sensitized with at least one merocyanine dye selected from those represented by the following general formula:



wherein R represents a primary alkyl group of the formula  $C_mH_{2m+1}$  wherein  $m$  represents a positive integer from 1 to 8,  $R_1$  represents a primary alkyl group of the formula  $C_qH_{2q+1}$  wherein  $q$  represents a positive integer from 1 to 20, L represents a methine group,  $d$  represents a positive integer from 1 to 3, and Z represents the non-metallic atoms necessary to complete a heterocyclic nucleus of the benzoselenazole series.

8. A photographic silver halide emulsion sensitized with at least one merocyanine dye selected from those represented by the following general formula:



wherein R represents a primary alkyl group of the formula  $C_mH_{2m+1}$  wherein  $m$  represents a positive integer from 1 to 8,  $R_1$  represents a primary alkyl group of the formula  $C_qH_{2q+1}$  wherein  $q$  represents a positive integer from 1 to 20, L represents a methine group,  $d$  represents a positive integer from 1 to 3, and Z represents the non-metallic atoms necessary to complete a heterocyclic nucleus of the thiazoline series.

9. A photographic silver halide emulsion sensitized with at least one merocyanine dye selected from those represented by the following general formula:



wherein R represents a primary alkyl group of the formula  $C_mH_{2m+1}$  wherein  $m$  represents a positive integer from 1 to 8,  $R_1$  represents a primary alkyl group of the formula  $C_qH_{2q+1}$  wherein  $q$  represents a positive integer from 1 to 20, L represents a methine group,  $d$  represents a positive integer from 1 to 3, and Z represents the non-metallic atoms necessary to complete a heterocyclic nucleus of the naphthothiazole series.

10. A photographic silver halide emulsion sensitized with at least one merocyanine dye selected from those represented by the following general formula:



wherein R represents a primary alkyl group of the formula  $C_mH_{2m+1}$  wherein  $m$  represents a positive integer from 1 to 8,  $R_1$  represents a primary alkyl group of the formula  $C_qH_{2q+1}$  wherein  $q$  represents a positive integer from 6 to 20,  $d$  represents a positive integer from 1 to 3, and Z 75

22

represents the non-metallic atoms necessary to complete a heterocyclic nucleus of the benzothiazole series.

5 11. A photographic silver halide emulsion sensitized with at least one merocyanine dye selected from those represented by the following general formula:



15 wherein R represents a primary alkyl group of the formula  $C_mH_{2m+1}$  wherein  $m$  represents a positive integer from 1 to 8,  $R_1$  represents a primary alkyl group of the formula  $C_qH_{2q+1}$  wherein  $q$  represents a positive integer from 6 to 20,  $d$  represents a positive integer from 1 to 3, and Z represents the non-metallic atoms necessary to complete a heterocyclic nucleus of the benzoxazole series.

12. A photographic silver halide emulsion sensitized with at least one merocyanine dye selected from those represented by the following general formula:



30 wherein R represents a primary alkyl group of the formula  $C_mH_{2m+1}$  wherein  $m$  represents a positive integer from 1 to 8,  $R_1$  represents a primary alkyl group of the formula  $C_qH_{2q+1}$  wherein  $q$  represents a positive integer from 6 to 20,  $d$  represents a positive integer from 1 to 3, and Z represents the non-metallic atoms necessary to complete a heterocyclic nucleus of the benzo-selenazole series.

40 13. A photographic silver halide emulsion sensitized with at least one merocyanine dye selected from those represented by the following general formula:



wherein R represents a primary alkyl group of the formula  $C_mH_{2m+1}$  wherein  $m$  represents a positive integer from 1 to 8,  $R_1$  represents a primary alkyl group of the formula  $C_qH_{2q+1}$  wherein  $q$  represents a positive integer from 6 to 20,  $d$  represents a positive integer from 1 to 3, and Z represents the non-metallic atoms necessary to complete a heterocyclic nucleus of the thiazoline series.

14. A photographic silver halide emulsion sensitized with the merocyanine dye represented by the following formula:



15. A photographic silver halide emulsion sensitized with the merocyanine dye having the following formula:



16. A photographic silver halide emulsion sensitized with the merocyanine dye represented by the following formula:



5

17. A photographic silver halide emulsion sensitized with the merocyanine dye represented by the following formula:



10

18. A photographic silver halide emulsion sensitized with the merocyanine dye represented by the following formula:



15

20

References Cited in the file of this patent

UNITED STATES PATENTS

| Number    | Name            | Date          |
|-----------|-----------------|---------------|
| 2,166,736 | White et al.    | July 18, 1939 |
| 2,177,402 | Brooker         | Oct. 24, 1939 |
| 2,263,749 | White et al.    | Nov. 25, 1941 |
| 2,282,116 | Brooker         | May 5, 1942   |
| 2,320,654 | Riester         | June 1, 1943  |
| 2,322,015 | Hamer et al.    | June 15, 1943 |
| 2,338,732 | Riester         | Jan. 11, 1944 |
| 2,340,832 | Kendall         | Feb. 8, 1944  |
| 2,353,164 | Kendall et al.  | July 11, 1944 |
| 2,656,353 | Jeffreys et al. | Oct. 20, 1953 |

OTHER REFERENCES

Chemical Abstracts 16:3101 (Abstract of Brit. Med. Journal, 1922 I 514-515).

Chemical Abstracts 19:530 (Abstract of Proc. Roy. Soc., London, 96B 317-333, 1924).